

Patented Sept. 22, 1925.

1,554,220

# UNITED STATES PATENT OFFICE.

CARL PIERCE LEWIS, OF BURLINGAME, CALIFORNIA, ASSIGNOR TO MINERALS SEPARATION NORTH AMERICAN CORPORATION, OF NEW YORK, N. Y., A CORPORATION OF MARYLAND.

## CONCENTRATION OF ORES.

No Drawing.

Application filed March 27, 1924. Serial No. 702,367.

To all whom it may concern:

Be it known that I, CARL PIERCE LEWIS, a citizen of the United States, and a resident of Burlingame, county of San Mateo, State of California, have invented certain new and useful Improvements in Concentration of Ores, of which the following is a specification.

This invention relates to the froth-flotation concentration of ores, and is herein described as applied to the concentration of certain ores with mineral-frothing agents in the presence of certain organic compounds containing sulphur.

It has been found that certain sulphur derivatives of carbonic acid greatly increase the efficiency of the froth-flotation process when used in connection with mineral-frothing agents. The increased efficiency shows itself sometimes in markedly better recoveries, sometimes in effecting the usual recoveries with greatly reduced quantities of the usual mineral-frothing agents, and sometimes in greatly reducing the time needed for agitation to produce the desired recoveries.

The invention is herein disclosed in some detail as carried out with salts of the sulphur derivatives of carbonic acid containing an organic radical, such as an alkyl radical, and known as xanthates as the new substance. These form anions and cations in solution. Excellent results were also obtained by agitating ore pulps with the complex mixture produced when 33 1/3% of pine oil was incorporated with an alcoholic solution of potassium hydrate, and xanthates or analogous substances were produced by adding carbon disulphide to this mixture.

The present application is in part a continuation of the application of Cornelius H. Keller and myself, filed October 23, 1923, Serial Number 670,242, which has been changed to a sole application of the said Cornelius H. Keller with claims for that part of the invention described and claimed in said joint application which was in fact the sole invention of the said Cornelius H. Keller. The present application claims that part of the invention described and claimed in said joint application which was in fact my sole invention.

According to the present invention these sulphur derivatives of carbonic acid may

be used in alkaline ore pulps or in ore pulps in which alkali has been added, and this or other procedure may be used to effect differential flotation of the various metaliferous minerals of complex ores.

The galena-bearing froth obtained with xanthates or analogous substances used at the rate of 0.2 pounds per ton of ore had a characteristic bright sheen, like a plumbago-bearing froth, and seemed to make a more coherent froth than when other materials were used on the same ore.

In general the substances referred to are not mineral-frothing agents, producing only a slight scum, and some evanescent frothy bubbles, when subjected to agitation which would produce mineral-bearing froth on an ore pulp in the presence of a mineral-frothing agent. The substances are effective in enabling a selective flotation of lead and zinc; and cause uncombined silver, if present, to tend to go into the lead concentrate rather than with the zinc, where these are separated in separate concentrates. Usually pre-agitation is unnecessary, the brightening and other effects seeming to be practically instantaneous.

For laboratory purposes potassium xanthate was prepared as follows:

198.4 grams of 88.5% caustic potash was dissolved in 524 grams ethyl alcohol (denatured #5 formula) at a temperature of 124° F., in a reflux condenser. The solution was cooled to 58° F. It contained a large excess of alcohol over the theoretical amount needed for the subsequent reactions. To this was added, while stirring, and in a cooling bath, the theoretical amount of carbon disulphide. The reaction was substantially instantaneous, producing a thick pulp of potassium xanthate. The pulp was cooled and centrifuged in a laboratory machine yielding crystals containing about 20% moisture. The yield thus obtained was 74.7%. Another 17.5% was obtained by evaporation of the mother liquor. Both the centrifuged crystals and the residue from the mother liquor gave excellent results in flotation. It was found in cases where sulphuric acid was used that the centrifuged material yielded better results than the uncentrifuged.

A pulp of Cash Mine ore subjected first to agitation for ten minutes with a mix-

ture of 0.3 pounds per ton of potassium xanthate with a small proportion of a 10% or a saturated solution of naphthalene in xylene, to yield a lead concentrate, and then 5 subjected to agitation for ten minutes with copper sulphate 0.2 pounds per ton, Barrett #4 flotation oil 1.0 pound per ton, and General Naval Stores #5 flotation oil 0.1 pounds per ton, yielded the results shown in the 10 following table. Attention is called to the recovery of 95% of the lead in a concentrate containing 87% of the silver but containing only 5% of zinc, while 70% of the zinc was recovered in the zinc concentrate.

15

*Cash Mine ore, assays.*

|              | %<br>Wt. | Au.<br>(oz.) | Ag.<br>(oz.) | Cu.  | Pb.  | Zn.  | Fe.  |
|--------------|----------|--------------|--------------|------|------|------|------|
| Heads.....   | 100.0    | .154         | 10.7         | 3.18 | 14.9 | 7.7  | 11.9 |
| Pb conc..... | 38.0     | .24          | 24.6         | 7.12 | 37.4 | 5.0  | 21.4 |
| Zn conc..... | 15.2     | .36          | 6.3          | 2.56 | 3.0  | 35.2 | 12.0 |
| Tails.....   | 46.6     | .015         | 0.9          | .26  | 0.5  | 0.8  | 4.2  |

*% RECOVERIES.*

25

|              | Au.  | Ag.  | Cu.  | Pb.  | Zn.  | Fe.  |
|--------------|------|------|------|------|------|------|
| Pb conc..... | 59.4 | 87.1 | 85.2 | 95.3 | 24.7 | 68.4 |
| Zn conc..... | 36.0 | 9.0  | 11.0 | 3.1  | 70.5 | 15.5 |
| Tails.....   | 4.6  | 3.9  | 3.8  | 1.6  | 4.8  | 16.4 |

30

A pulp of San Francisco Mines of Mexico ore was agitated for ten minutes with potassium xanthate 0.15 pounds per ton and the same amount of coal tar creosote to yield a lead concentrate. The remaining pulp was agitated for fifteen minutes with 0.2 pounds per ton of copper sulphate, 1.2 pounds per ton of water-gas tar, and 0.05 pounds per ton of steam distilled pine oil. 35 The results are shown in the following table:

*San Francisco Mines of Mexico.*

|              | Assays. |              |      |      | % Recoveries. |      |      |
|--------------|---------|--------------|------|------|---------------|------|------|
|              | % Wt.   | Ag.<br>(oz.) | Pb.  | Zn.  | Ag.           | Pb.  | Zn.  |
| Heads.....   | 100.0   | 16.5         | 9.4  | 16.1 |               |      |      |
| Pb conc..... | 12.2    | 67.0         | 64.0 | 12.0 | 49.4          | 83.2 | 9.1  |
| Zn conc..... | 28.9    | 23.6         | 3.6  | 43.4 | 41.2          | 11.1 | 78.0 |
| Tails.....   | 58.9    | 4.5          | 1.5  | 6.0  | 9.4           | 5.7  | 12.9 |

Similar results were obtained with this ore by agitating for five minutes with 0.15 pounds each of sodium xanthate and Barrett No. 2 flotation oil per ton of ore, to yield a lead concentrate, and then agitating for ten minutes with 0.3 pounds copper sulphate, 1.3 pounds Barrett No. 4 flotation oil, and General Naval Stores No. 5 flotation oil 0.1 pounds, all per ton of ore, to yield a zinc concentrate.

Anaconda ore slimes containing 3.28% copper of which 0.45% was acid soluble, were subjected to froth-flotation concentration at 70° F. with 7.8 pounds per ton of

dry hydrated lime, 0.132 pounds per ton of steam distilled pine oil 0.38 pounds per ton of destructively distilled pine oil (G. N. S. #11 flotation), and 0.69 pounds per ton of potassium xanthate in solution, yielding 70 concentrates containing 13.76% copper and 34.7% insolubles, with a tailing of 0.317% copper of which 0.173% was acid soluble. This represented a recovery of 92.2%.

The lime was mixed with water and fed 75 as a watery paste with the slimes to the first agitator of a series of nine standard minerals separation agitators or mixing compartments through which the pulp passed in series at the rate of 97 tons in 80 24 hours. The #11 pine oil was added at the seventh agitator and 0.6 pounds per ton of the xanthate at the ninth. The pulp returned through fourteen spitzkastens each 85 equipped with a Brown aerator and circulating device. At the sixth spitzkasten the balance of the xanthate was added. At the tenth spitzkasten the steam distilled pine oil was added. The froth from the first nine spitzkastens was collected as a 90 finished concentrate, that from the remaining five was returned to the first as a middling.

It has also been found that for the froth-flotation concentration of certain ores, such 95 as Calumet & Hecla, Britannia, Cananea and Moctezuma, mother liquor obtained from centrifuging the above described xanthates in the process of manufacture of said xanthates may be used with about the same 100 proportions of mother liquor as of the xanthate crystals specified with results as good or better than those above given.

In one test a freely flowing pulp containing 1200 grams of Anaconda slimes assaying 2.95% copper was agitated 15 minutes in a sub-aeration machine at 17° C. with 5 pounds of soda ash, 0.7 pounds of potassium xanthate, and 0.2 pounds of steam distilled pine oil, all per ton of ore, yielding a concentrate containing 13.68% copper. The ratio of concentration was 5.2. The 110 concentrate contained 91.5% of the copper, and an additional 4.1% was contained in a middling which held 0.68% of copper. The tailings contained 0.20% of copper which was 4.4% of that present in the heads.

The xanthate may be used to replace a part of the alkali normally used in the concentration of certain ores, and in differential flotation it may be used to replace either a part or all of the alkali normally used.

A pulp of Park Utah lead-zinc ore was 120 agitated for ten minutes with potassium xanthate 0.15 pounds, and Barrett #2 flotation oil 0.15 pounds, to yield a lead concentrate. The remainder of the pulp was then agitated fifteen minutes with soda ash, 1.5 pounds, copper sulphate, 0.5 pounds,

water gas tar, 1 pound, and pine oil, 0.05 pounds, to yield a zinc concentrate. The zinc concentrate was then reagitated with added water for five minutes to yield a finished zinc concentrate and a zinc middling. All flotation and frothing agents were measured in pounds per ton. The results are shown in the following table:

| 10           | % Assays. |              |      |       | Recoveries. |      |      |
|--------------|-----------|--------------|------|-------|-------------|------|------|
|              | % Wt.     | Ag.<br>(oz.) | Pb.  | Zn.   | Ag.         | Pb.  | Zn.  |
| Heads.....   | 100.0     | 5.39         | 8.24 | 12.55 | 68.0        | 85.2 | 9.7  |
| Pb conc..... | 11.7      | 31.3         | 60.0 | 10.4  |             |      |      |
| Zn conc..... | 29.3      | 4.2          | 1.7  | 32.0  | 22.8        | 6.1  | 75.3 |
| Zn midd..... | 3.0       | 3.6          | 3.5  | 12.4  | 2.0         | 1.3  | 4.6  |
| Tails.....   | 56.0      | 0.7          | 1.1  | 2.3   | 7.2         | 7.4  | 10.4 |

A pulp of Sullivan ore was agitated for seven minutes with potassium xanthate 0.1 pounds, and coal tar creosote, 0.1 pounds, to yield a lead concentrate. The remaining pulp was then agitated fifteen minutes with soda ash, 2 pounds, sulphate of copper, 0.5 pounds, and water gas tar, 1.3 pounds, to yield a zinc concentrate. All these quantities were in pounds per ton of ore. These concentrates were reagitated with the addition of water to produce respectively a lead finished concentrate and middling and a zinc finished concentrate and middling. The results are shown in the following table:

| 35           | % Assays. |              |       |      | % Recoveries. |      |      |      |
|--------------|-----------|--------------|-------|------|---------------|------|------|------|
|              | % Wt.     | Ag.<br>(oz.) | Pb.   | Zn.  | Fe.           | Pb.  | Zn.  | Fe.  |
| Heads.....   | 100.0     | 13.1         | 12.06 | 15.3 | 30.6          | 75.2 | 9.0  | 4.0  |
| Pb conc..... | 15.0      | 60.4         | 9.2   | 8.2  |               |      |      |      |
| Pb midd..... | 5.3       | 3.6          | 15.6  | 12.0 | 35.5          | 6.8  | 4.2  | 6.0  |
| Zn conc..... | 29.3      | 2.1          | 6.0   | 43.0 | 13.3          | 14.4 | 82.4 | 12.6 |
| Zn midd..... | 4.6       | 1.1          | 3.6   | 6.4  | 45.2          | 1.4  | 2.0  | 6.8  |
| Tails.....   | 45.8      | 0.4          | .6    | .8   | 47.2          | 2.2  | 2.4  | 70.6 |

A pulp of the highly refractory ore of the North Star Mine of the Federal Mining & Smelting Co. was agitated for ten minutes with an added mixture of 90% potassium xanthate and 10% Barrett No. 2 creosote, 0.2 pounds, and with 0.1 pounds of separately added Barrett No. 2 creosote, to yield a lead concentrate. The remaining pulp was reagitated for fifteen minutes with copper sulphate, 0.7 pounds, soda ash, 1.5 pounds, Barrett No. 4 flotation oil, 1.4 pounds, to yield a zinc concentrate. All weights are per ton of ore. The results are shown in the following table:

| 60           | % Assays. |              |      |      | % Recoveries. |      |      |      |      |
|--------------|-----------|--------------|------|------|---------------|------|------|------|------|
|              | % Wt.     | Ag.<br>(oz.) | Pb.  | Zn.  | Fe.           | Ag.  | Pb.  | Zn.  | Fe.  |
| Heads.....   | 100.0     | 10.1         | 7.9  | 18.4 | 14.8          |      |      |      |      |
| Pb conc..... | 13.7      | 37.4         | 31.2 | 10.8 | 13.2          | 50.7 | 64.9 | 8.0  | 12.2 |
| Zn conc..... | 57.7      | 7.9          | 5.0  | 27.0 | 17.0          | 45.0 | 36.9 | 84.9 | 66.2 |
| Tails.....   | 28.6      | 1.5          | 2.5  | 4.6  | 11.2          | 4.3  | 8.2  | 7.1  | 21.7 |

A pulp of 80 mesh Calumet and Hecla slimes containing 0.44% copper, mostly native, with considerable mineral occluded in the coarser particles of the gangue, was agitated for twenty-five minutes with caustic soda 1 pound, potassium xanthate 0.25 pounds, N. T. U. oil 0.25 pounds, and 0.25 pounds pine oil and rosin mixed, all in pounds per ton. The results are shown in the following table:

|            | % Assays. |       |       | % Recoveries. |    |
|------------|-----------|-------|-------|---------------|----|
|            | % Wt.     | Cu.   | Cu.   | Cu.           | 80 |
| Heads..... |           | 100.0 | 0.44  |               |    |
| Conc.....  |           | 1.6   | 12.24 | 44.8          |    |
| Midd.....  |           | 21.4  | 0.88  | 43.2          |    |
| Tails..... |           | 77.0  | 0.068 | 12.0          |    |

85

Other tests indicated that in commercial operations it would be possible to take off a concentrate containing 30% to 40% of copper, returning some or all the remainder of the concentrate as a middling for retreatment or diverting it to separate treatment.

To preferentially float copper and not iron it has been found advantageous to add lime or slaked lime during fine grinding so that the pulp shows an alkalinity of 0.5% to 1% in the filtrate from the ore pulp when titrated against  $\frac{1}{4}$   $\text{NH}_3\text{SO}_4$  using phenolphthalein as indicator. Pulp thus treated when subjected to agitation with 0.1 to 0.15 pounds of a xanthate per ton and a minimum of mineral-frothing agents selects copper over iron more effectively than has hitherto been possible.

Phelps-Dodge table concentrates were ground with 5 pounds of lime per ton to make about 300-mesh material and then agitated in a pulp for five minutes with potassium xanthate, 0.10 pounds per ton, and steam distilled pine oil, 0.05 pounds per ton, to yield a concentrate. The pulp was then further agitated for fifteen minutes with an addition of potassium xanthate, 0.05 pounds per ton, and the same pine oil, 0.05 pounds per ton, to yield a middling. The results are shown in the following table:

|            | % Assays. |       |       | % Recoveries. |      |
|------------|-----------|-------|-------|---------------|------|
|            | % Wt.     | Cu.   | Cu.   | Cu.           | 120  |
| Heads..... |           | 100.0 | 3.71  |               |      |
| Conc.....  |           | 8.5   | 26.88 | 31.4          | 61.7 |
| Midd.....  |           | 9.4   | 8.68  | 40.7          | 22.0 |
| Tails..... |           | 82.1  | .74   | 43.3          | 16.3 |

125

It will be noted that there was effective concentration of the copper, but no concentration of the iron even in this highly refractory ore.

130

Having thus described certain embodiments of this invention what is claimed is:

1. The improvement in the concentration of minerals by flotation which comprises subjecting the mineral in the form of an alkaline pulp to a flotation operation in the presence of a xanthate.

2. The improvement in the concentration of minerals by flotation which comprises subjecting the mineral in the form of a pulp made alkaline by the addition of lime to a flotation operation in the presence of a xanthate.

3. The improvement in the concentration of minerals by flotation which comprises subjecting the mineral in the form of an alkaline pulp to a flotation operation in the presence of potassium xanthate.

4. The improvement in the concentration of minerals by flotation which comprises subjecting the mineral in the form of a pulp made alkaline by the addition of lime to a flotation operation in the presence of potassium xanthate.

5. The improvement in the concentration of minerals by flotation which comprises subjecting the mineral in the form of an alkaline pulp to a flotation operation in the presence of potassium xanthate and a frothing agent.

6. The process of concentrating an ore which consists in agitating a pulp of the ore with a sulphur derivative of carbonic acid adapted to yield anions and cations in solution and with a mineral-frothing agent to form a mineral-bearing froth and separating the froth.

7. The process of concentrating an ore which consists in agitating an alkaline pulp of the ore with a sulphur derivative of carbonic acid adapted to yield anions and cations in solution and with a mineral-frothing agent to form a mineral-bearing froth and separating the froth.

8. The process of concentrating a complex ore which consists in agitating a pulp of the ore with a sulphur derivative of carbonic acid adapted to yield anions and cations in solution and with a mineral-frothing agent to form a mineral-bearing froth relatively rich in one mineral; separating the froth, further agitating the pulp with further added flotation agent to form a mineral-bearing froth relatively rich in another mineral, and separating the second froth.

9. The process of concentrating a complex ore which consists in agitating a pulp of the ore with a sulphur derivative of carbonic acid adapted to yield anions and cations in solution and with a mineral-frothing agent to form a mineral-bearing froth relatively rich in one mineral, separating the froth, further agitating the pulp

with the addition of flotation agent including an alkaline substance to form a mineral-bearing froth relatively rich in another mineral, and separating the second froth.

10. The process of concentrating an ore which consists in agitating a pulp of the ore with a xanthate and a mineral-frothing agent and an added alkaline substance to form a mineral-bearing froth and separating the froth.

11. The process of concentrating a complex ore which consists in agitating a pulp of the ore with a xanthate and a mineral-frothing agent to form a mineral-bearing froth relatively rich in one mineral, separating that froth, and further agitating the pulp with further added mineral-frothing agent to form a second mineral-bearing froth relatively rich in another mineral, and separating the second froth.

12. The process of concentrating a complex ore which consists in agitating a pulp of the ore with a xanthate and a mineral-frothing agent to form a mineral-bearing froth relatively rich in one mineral, separating that froth, further agitating the pulp with an alkaline substance to form a second mineral-bearing froth relatively rich in another mineral and separating the second froth.

13. The process of concentrating a complex ore which consists in agitating a pulp of the ore with a xanthate and a mineral-frothing agent to form a mineral-bearing froth relatively rich in one mineral, separating that froth, further agitating the pulp with added flotation agent including an alkali to form a second mineral-bearing froth relatively rich in another mineral, and separating the second froth.

14. The process of concentrating a lead-zinc ore which consists in agitating a pulp of the ore with a xanthate and a mineral-frothing agent to form a lead-bearing froth, separating the froth, further agitating the pulp with further added mineral-frothing agent to form a zinc-bearing froth, and separating the second froth.

15. The process of concentrating an ore which consists in agitating a pulp of the ore with a sulphur derivative of carbonic acid containing an organic radical and with a mineral-frothing agent and an added alkaline substance to form a mineral-bearing froth, and separating the froth.

16. The process of concentrating an ore which consists in agitating an alkaline pulp of the ore with a sulphur derivative of carbonic acid containing an organic radical and with a mineral-frothing agent to form a mineral-bearing froth, and separating the froth.

In testimony whereof, I have affixed my signature to this specification.

CARL PIERCE LEWIS.